

## UNITED STATES PATENT OFFICE

2,481,424

METHOD OF PRODUCING BLACK OXIDE  
COATED STEEL SHEETS

John W. Hill, Mansfield, Ohio, assignor, by mesne assignments, to Empire Steel Company, a corporation of Delaware

No Drawing. Application October 11, 1946,  
Serial No. 702,578

14 Claims. (Cl. 148—6.35)

1.

This invention relates, as indicated, to a method of producing coated sheets, but has reference more particularly to the production of oxide-coated steel sheets.

A primary object of the invention is to produce a steel sheet having an oxide coating, which is extremely attractive in appearance, and which is both heat and corrosion resistant.

Another object of the invention is to provide an oxide-coated steel sheet of the character described which can be bent, formed, drawn, or otherwise fabricated without breakage of the oxide film or coating.

A further object of the invention is to provide an oxide-coated steel sheet of the character described which is especially adapted for use in the production of stoves, refrigerators, and other household equipment, but which is adapted for other uses.

Other objects and advantages of the invention will be apparent during the course of the following description.

In accordance with the invention, steel sheets are first placed in an annealing box, and piled in such box to a desired height, the box being then covered in accordance with conventional pile or box annealing practice.

The pile of sheets is then heated to an annealing temperature within the range of from about 800° F. to about 1200° F., the anneal being continued until the sheets at the bottom of the pile attain the said annealing temperature. In practice, the annealing period is from about 10 to about 20 hours, depending upon the size and number of sheets in the pile. During this anneal, a deoxidizing gas of any desired analysis is passed through the annealing box.

At the end of the aforesaid heating period, the heating of the pile is discontinued, and before the temperature of the pile has dropped below about 700° F., steam is introduced into the annealing box, causing a blue oxide coating to be formed on both surfaces of each sheet, and when the temperature of the pile has fallen below about 250° F., the passage of steam into the box is discontinued.

The cover of the box is then removed, and the sheets permitted to cool to atmospheric temperatures.

The aforesaid treatment is thus a combination of a conventional anneal, and a coating of the sheet surfaces with a film or coating of a blue oxide, which I term a "steam blue oxide."

The sheets are then removed from the annealing box, and are then cold-rolled to impart smoothness to the oxide-coated surfaces of the sheets.

The cold-rolled sheets are then passed through a coating machine containing petroleum asphalt, which is a mixture of hydrocarbons and complex organic compounds derived from still residues

when asphalt-base petroleum is refined. For this particular purpose, the petroleum asphalt is preferably diluted with kerosene in an amount equal to one-third by volume of the coating solution.

The sheets, which have thus been provided with a coating of petroleum asphalt, are then run through a conveyor-type furnace, in which they are heated to a temperature within the range of from about 500° F. to about 700° F., which is the flash or ignition temperature of the petroleum asphalt-kerosene coating, and at this temperature, the coating becomes ignited and burns with a luminous yellow flame. The entire combustion of the coating requires about thirty seconds, and at the conclusion thereof, the sheets are run out of the furnace and onto a sheet piler.

The effect of the combustion of the petroleum asphalt or petroleum asphalt-kerosene solution is to reduce the "steam blue oxide" to an iron oxide of lower oxygen content, which is jet black in color, and the physical appearance of which depends on the nature of the original surface of the steel sheet. If the steel sheet had a smooth, mirror-like finish, the black oxide of the finished sheet will be highly lustrous in appearance. If the steel sheet had a roughened or matte-like surface, the black oxide will have a matte-like appearance.

30 The finished product or sheet is extremely attractive in appearance and is highly resistant to heat as well as corrosion. It can be readily bent, formed, drawn or otherwise fabricated, without breakage of the oxide film or coating.

35 By virtue of these properties, it is admirably adapted for use in the production of stoves, refrigerators, and other household equipment, but is well adapted for numerous other applications or uses.

40 Instead of box or pile annealing the sheets, as described, the sheets may be run through a continuous annealing furnace and heated to the desired annealing temperature, and after the sheets have attained this temperature, steam may be introduced into the furnace in order to form the blue oxide coating to which reference has been made.

Moreover, the process is adapted for the treatment of strip steel in a continuous manner. The coil of strip steel may either be box-annealed and coated with the blue oxide, and the strip then run, in a continuous manner, through the coating machine and coating-burning furnace, or the strip may be run, in a continuous manner, through a continuous annealing furnace, in which it is annealed and coated with the blue oxide, and then run, in a continuous manner, through the coating machine and coating-burning furnace.

60 It will be understood that various changes in

temperatures, strengths of solutions, and other details of the method may be resorted to, without departing from the scope of the subjoined claims.

Having thus described my invention, I claim:

1. In a method of producing heat and corrosion resistant steel sheets, the steps which consist in forming a blue oxide coating on said sheets, coating said sheets with petroleum asphalt, and igniting said petroleum asphalt, whereby said coating burns and said blue oxide is reduced to a black oxide.

2. In a method of producing heat and corrosion resistant steel sheets, the steps which consist in forming a blue oxide coating on said sheets, coating said sheets with a solution of petroleum asphalt and kerosene, and then igniting the asphalt and kerosene, whereby the asphalt and kerosene burn and said blue oxide is reduced to a black oxide.

3. In a method of producing heat and corrosion resistant steel sheets, the steps which consist in simultaneously annealing said sheets and forming a blue oxide coating thereon, coating said sheets with petroleum asphalt, and igniting said petroleum asphalt, whereby said asphalt burns and said blue oxide is reduced to a black oxide.

4. In a method of producing heat and corrosion resistant steel sheets, the steps which consist in simultaneously annealing said sheets and forming a blue oxide coating thereon, coating said sheets with a mixture of petroleum asphalt and kerosene, and igniting the asphalt and kerosene, whereby the asphalt and kerosene burn and said blue oxide is reduced to a black oxide.

5. In a method of producing heat and corrosion resistant steel sheets, the steps which consist in heating said sheets, subjecting the heated sheets to the action of steam, whereby a blue oxide coating is formed on said sheets, coating said sheets with petroleum asphalt, and igniting said petroleum asphalt, whereby said asphalt burns and said blue oxide is reduced to a black oxide.

6. In a method of producing heat and corrosion resistant steel sheets, the steps which consist in heating said sheets to a temperature within the range of from about 800° F. to about 1200° F., subjecting the hot sheets before they have cooled below about 700° F. to the action of steam, whereby a blue oxide coating is formed on said sheets, coating said sheets with petroleum asphalt, and igniting said petroleum asphalt, whereby said asphalt burns and said blue oxide is converted to a black oxide.

7. A method, as defined in claim 6, in which the sheets are heated in a deoxidizing atmosphere.

8. A method, as defined in claim 6, in which the sheets are cold-rolled before being coated with petroleum asphalt.

9. In a method of producing heat and corrosion resistant steel sheets, the steps which consist in heating said sheets to a temperature within the range of from about 800° F. to about 1200° F., subjecting the sheets before they have cooled below about 700° F. to the action of steam, whereby a blue oxide-coating is formed on the sheets, coating said sheets with petroleum asphalt, and heating the sheets to a temperature at which said last-named coating becomes ignited and burns with a luminous flame until it is consumed, the combustion of said petroleum asphalt coating converting said blue oxide coating to a coating which is black in color.

10. A method, as defined in claim 9, in which the sheets are cold-rolled before being coated with petroleum asphalt.

11. A method, as defined in claim 9, in which the first heating of the sheets is conducted in a deoxidizing atmosphere.

12. A method of producing heat and corrosion resistant steel sheets, comprising the steps of piling the sheets in an annealing box, covering said box, heating the pile to a temperature within the range of from about 800° F. to about 1200° F., passing a deoxidizing gas into said box during the heating period, discontinuing said heating, passing steam into the box before the temperature of the pile has been reduced below about 700° F., thereby forming a blue oxide coating on the sheets, cutting off the flow of steam when the temperature of the pile has fallen to about 250° F., removing the cover from said box, permitting the sheets to cool to atmospheric temperature, removing the sheets from said box, cold-rolling the sheets to impart smoothness to the coating, coating the sheets with petroleum asphalt, passing the sheets through a furnace in which the sheets are heated to a temperature at which the petroleum asphalt is ignited and burns with a luminous flame until the petroleum asphalt is spent, said combustion resulting in a conversion of said blue oxide coating to a black coating.

13. In a method of producing heat and corrosion resistant steel sheets, the steps which consist of applying to sheets having a blue oxide coating thereon a coating of petroleum asphalt, and igniting said asphalt whereby the asphalt burns and said blue oxide is reduced to a black oxide.

14. In a method of producing heat and corrosion resistant steel sheets, the steps which consist of applying to sheets having a blue oxide coating thereon a coating of petroleum asphalt, and heating the sheets to a temperature at which the asphalt coating becomes ignited and burns with a luminous flame until it is consumed, the combustion of said asphalt coating converting said blue oxide coating to a coating which is black in color.

JOHN W. HILL.

#### REFERENCES CITED

50 The following references are of record in the file of this patent:

#### UNITED STATES PATENTS

| Number    | Name            | Date          |
|-----------|-----------------|---------------|
| 234,524   | Bower, et al.   | Nov. 16, 1880 |
| 406,858   | Schmid          | July 9, 1889  |
| 798,365   | Rupley          | Aug. 29, 1905 |
| 881,221   | Bontempi        | Mar. 10, 1908 |
| 1,056,627 | Carnahan et al. | Mar. 18, 1913 |
| 1,346,473 | Swan            | July 13, 1920 |
| 2,196,172 | Billings et al. | Apr. 9, 1940  |
| 2,201,981 | Baron           | May 28, 1940  |
| 2,333,936 | Johnson         | Nov. 9, 1943  |

#### OTHER REFERENCES

65 Abraham, "Asphalts and Allied Substances," fifth edition (1945), vol. I, page 463, Van Nostrand Co., Inc., New York.

70 H. Silman, Metal Industry, May 25, 1945, pages 330 to 332.